

1,140,898.

W. GIBSON, SR. & R. SKEMP.  
METHOD OF GALVANIZING.  
APPLICATION FILED MAR. 9, 1912.

Patented May 25, 1915.  
2 SHEETS—SHEET 1.



FIG. 1

**WITNESSES**

W. T. Stolman

R. D. Little

**INVENTORS**

William Gibson Sr.

Robert Skemp  
64 Ludicium Beta, Fuller  
their attorney

1,140,898.

W. GIBSON, SR. & R. SKEMP,  
METHOD OF GALVANIZING,  
APPLICATION FILED MAR. 9, 1912.

Patented May 25, 1915.

2 SHEETS—SHEET 2.



FIG. 2



FIG. 3

WITNESSES

*W.T. Holman*

*R. Little*

INVENTORS

William Gibson, Sr  
Robert Skemp  
Lithuanian Bell & Ball  
their Attorneys

# UNITED STATES PATENT OFFICE.

WILLIAM GIBSON, SR., OF VANDERGRIFT, AND ROBERT SKEMP, OF SCOTTDALE, PENNSYLVANIA, ASSIGNORS TO AMERICAN SHEET & TIN PLATE COMPANY, OF PITTSBURGH, PENNSYLVANIA, A CORPORATION OF NEW JERSEY.

## METHOD OF GALVANIZING.

1,140,898.

Specification of Letters Patent. Patented May 25, 1915.

Application filed March 9, 1912. Serial No. 682,666.

*To all whom it may concern:*

Be it known that we, WILLIAM GIBSON, Sr., and ROBERT SKEMP, both citizens of the United States, residing at Vandergrift, in the county of Westmoreland and State of Pennsylvania, and Scottdale, in the county of Westmoreland and State of Pennsylvania, respectively, have invented a new and useful Method of Galvanizing, of which the following is a specification.

Our invention relates to the coating of metal and more particularly relates to the galvanizing of metal sheets and plates.

Heretofore in coating metals by existing methods, great difficulty has been experienced in keeping the surface of the molten metal or metal alloy, through which the sheets or other articles pass, free from oxidation and in a free flowing condition as the articles leave the galvanizing pot. When the articles are mechanically conveyed through the pot, the surfaces of the exit rolls become covered more or less with metallic oxid which adheres to the sheets in patches, and prevents the desired uniform distribution of the coating. The coating on the sheets or other articles also is liable to rapid oxidation while still molten, such oxidation preventing a uniform flow of the coating on the coated article and also acting to give a dull appearance to the surfaces of the coating.

One object of our invention is to provide a novel method of coating iron and steel sheets or other articles whereby the formation and accumulation of films or layers of metallic oxid on the surface of the molten metal is to a considerable extent prevented and overcome, and damage to the coated materials delivered from the galvanizing pot or other receptacle containing the molten coating is avoided.

Another object of our invention is to secure fluidity and prevent oxidation of the molten metal on the surfaces of the sheets or other articles being coated, and thereby secure uniformity of coating and obtain the desired lustrous appearance of the coated materials.

A further object of this invention is to provide novel means whereby the steps of our improved method are carried out or effected.

Still further objects of the invention will

appear, as the invention is more fully described hereinafter.

Our invention is applicable for use in galvanizing by handling the materials manually in dipping and withdrawing the materials being coated from the bath of molten metal, as well as to galvanizing by the aid of mechanical means. As the latter process is in more general use, the accompanying drawings forming part of this specification have been described with reference to the coating of metals by the aid of mechanical means employed in conveying the sheets or other articles into and through the bath of molten metal or alloyed metals forming the coating material.

In the accompanying drawings, Figure 1 is a plan showing a galvanizing pot having conveying mechanism mounted therein by which the materials being coated are caused to enter, pass through and emerge from the galvanizing pot, and having apparatus mounted thereon by which our improved process is carried out. Fig. 2 is an elevation, on an enlarged scale, showing the apparatus forming part of this invention as applied for use on the galvanizing pot in carrying out the steps of our improved process. Fig. 3 is a longitudinal sectional elevation taken on the line III—III of Fig. 2.

In the drawings, the numeral 2 designates a galvanizing pot having feed-in rolls 3 and 4, and feed-out rolls 5 and 6. The guides employed in connection with the feed-in and feed-out rolls in conveying the materials through the pot are omitted for the sake of clearness.

Secured on one end of the galvanizing pot 2 by the knee 7 so as to be located to one side of the pot 2 is the grinding or pulverizing mechanism 8 and in the hopper 9 of the grinding mechanism a supply of sal-ammoniac or other suitable fluxing material is maintained, which is ground and fed in regulated quantities into the funnel or hopper 10 located below the delivery opening 11 in the grinding mechanism 8 when the mechanism is actuated by the belt connecting the pulley 19 thereon with the pulley driving mechanism. The lower, smaller end 105 of the hopper 10 projects through an opening in the top of the shield or hood 23 which is arranged to extend over the side of the

galvanizing pot 2. The bottom opening 12 in the funnel 10 is located to one side of the exit or feed-out rolls 5 and 6 and in vertical alinement with the contacting faces 5 of these rolls.

On one side of the galvanizing pot 2 is a horizontally extending pipe or conduit 13 having an opening 14 in one end. The axial center of this pipe, the center of the outlet 10 opening 12 in the funnel 10 and the line of contact between the surfaces of the feed-out rolls 5 and 6 are all in the same vertical plane and a valve 15 is provided on the pipe or conduit 13 to regulate and control the 15 supply of compressed air or other gaseous fluid delivered therethrough.

The grinding mechanism 8 has a worm 16 therein which is mounted in bearings 17 and 18 and a driven pulley 19 on the outer 20 end of the worm 16 is connected by a belt 20 to a driving pulley 21 secured on the counter-shaft 22. The counter-shaft 22 preferably is connected by a belt or other suitable means with the driving mechanism 25 for the feed rolls in the galvanizing pot 2 although separate driving means may be employed for the grinding mechanism when found necessary or desirable.

In carrying out the steps of our improved 30 method, the feed-in rolls 3 and 4 and feed-out rolls 5 and 6 are operated in the usual manner in carrying plates or sheets into and through the bath of molten spelter or other coating material maintained in the 35 pot.

Carbon dioxid or other substantially dry non-oxidizing gas is supplied under pressure through the pipe 13 to the galvanizing pot 2, a stream of the gaseous fluid issuing from 40 the opening 14 in the end of the pipe 13. The stream of gaseous fluid is caused to pass through the open end 24 of the shield or cover 23 and across the face of the feed-out rolls 5 and 6 on the exit side of the pot 45 2 so that the sheets and plates or other materials in emerging from the pot issue from between these rolls into an atmosphere consisting in whole or in part of non-oxidizing gases. The grinding mechanism 8 being operated when the galvanizing pot 2 is in operation, the sal-ammoniac or other fluxing agent placed in the hopper 9 is ground and a steady stream of finely divided flux is gradually fed through the exit opening 11 50 into the funnel 10. The funnel 10 directs the regulated quantities of the fluxing agent into the path of the stream of gases issuing from the opening 14 in the end of the pipe 13 and is carried thereby over the surface 55 of the metal between the feed-out rolls 5 and 6, on the exit side of these rolls, and across the coated surfaces of the articles emerging from between the feed-out rolls.

The particles of sal-ammoniac or other fluxing agent act to decompose any metallic

oxid which may have been formed on the molten metal at the point of exit of the coated material from the galvanizing pot or on the surfaces of the molten coating adhering to the coated material emerging from the pot and act to produce a fluidity of the coating metal adhering to the coated surfaces of the emerging materials, which insures a uniform and complete distribution of the molten coating over the surfaces of the material being coated.

The advantages of our invention will be apparent to those skilled in the art.

By supplying finely divided sal-ammoniac or other fluxing agent to the surface of the molten metal at the exit end of the galvanizing pot and by supplying finely divided fluxing agent to the molten coating on the coated material emerging from the pot, the coating metal is maintained in a fluid condition and a uniform distribution of the coating is secured with an absence of list on the ends or edges of the coated material.

The sheets or other articles being coated are caused to emerge from the molten bath of galvanizing metal into an atmosphere formed wholly or partially of dry non-oxidizing gases and the coating metal is thereby kept from oxidation, the luster of the coating is preserved and an improved material is obtained.

Modifications in the construction and arrangement of the apparatus and changes in the steps of the method may be made without departing from our invention.

Air or other gaseous fluid pressure may be used instead of carbon dioxid to propel or impinge the fluxing agent across the face of the metal at the feed-out rolls on the exit side thereof and across the surfaces of material emerging from the pot.

The means employed in supplying the finely divided fluxing agent to the feed-out rolls or point of exit from the pot, and across the surfaces of articles coated may be varied and other changes may be made. Zinc chlorid and other fluxing agents may be employed in carrying out the steps of our improved method within the scope of the appended claims.

We claim:—

1. The method of coating sheets and similar metal articles which consists in conveying the articles through a molten bath of coating metal, and impinging a finely divided fluxing agent upon the molten surfaces of the coating on the articles as the articles leave the bath of coating metal, to thereby prevent oxidation and secure a uniform distribution of the coating metal on the surfaces of the coated articles.

2. The method of coating sheets and similar metal articles which consists in conveying the articles through a molten bath of

- coating metal into an atmosphere of at least partially non-oxidizing gases and simultaneously applying a finely divided fluxing agent upon the molten surfaces of the coating metal on the articles as the articles leave the bath of coating metal, to thereby prevent oxidation and secure a uniform distribution of the molten coating metal on the surfaces of the coated articles.
3. The method of coating sheets and the like which consists in mechanically conveying the articles through a molten bath of coating metal, causing the coated articles to emerge therefrom into an atmosphere at least partially formed of non-oxidizing gases, and impinging a finely divided fluxing agent on the molten surfaces of the coating upon the articles emerging from the pot and to the uppermost surfaces of the feed-out rolls during the coating operations, to thereby prevent oxidation of the coating and secure a uniform distribution of the coating metal on the surfaces of the coated materials.
4. The method of coating sheets and other articles, which consists in mechanically passing the sheets through the molten coating metal and impinging a finely divided fluxing agent on the surface of the molten coating on the articles and the uppermost surfaces of the feed-out rolls at the exit end of the pot during the coating operations to thereby prevent oxidized coating metal adhering to the surfaces of said feed-out rolls.
5. The method of coating sheets or plates consisting in passing the materials into and through the bath of coating metal, feeding the sheets out of the bath of coating metal by means of feed-out rollers, feeding regulated quantities of a suitable fluxing agent during the coating operations to the surface of the molten coating on the coated materials at the exit end of the pot and the surfaces of the feed-out rolls by blowing the finely divided flux across the uppermost faces of the rolls and across the surfaces of the articles emerging from the pot by means of a blast of gaseous fluid pressure.
6. The method of coating sheets or plates consisting in passing the materials into and through the bath of coating metal in feeding the sheets out of the bath of coating metal by means of feed-out rollers, blowing a stream of gases across the exit end of the pot to create an atmosphere of at least partially non-oxidizing gases into which the sheets emerge from the pot and utilizing the force of the stream of gases to distribute a finely divided flux on the surface of the molten metal, the faces of the rolls and across the fluid coating on the coated articles to prevent oxidation of the coating and produce fluidity of the coating metal and thereby secure uniform distribution of the coating on the coated materials.
7. The method of coating sheets and other articles consisting in passing the materials into and through the bath of coating metal, blowing a stream of gases across the molten metal at the exit end of the pot to create an at least partly non-oxidizing atmosphere into which the coated materials emerge, feeding a finely divided fluxing agent in regulated quantities into the path of the stream of gases and utilizing the force of the stream of gases to distribute the finely divided flux on the molten metal at the exit end of the pot to prevent oxidization and secure fluidity of the coating metal on the surface of the coated materials and thereby secure a uniform coating free from breaks and patches, and of a lustrous appearance.
- In testimony whereof, we have hereunto set our hands.
- WILLIAM GIBSON, SR.  
ROBT. SKEMP.
- Witnesses to the signature of William Gibson, Sr.:
- FRANK T. MCGINNIS,  
CHAS. J. WILLEMBERG.
- Witnesses to the signature of Robt. Skemp:
- G. C. KIMBALL,  
S. B. YOARBY.

It is hereby certified that in Letters Patent No. 1,140,898, granted **May 25, 1915**, upon the application of William Gibson, Sr., of Vandergrift, and Robert Skemp, of Scottdale, Pennsylvania, for an improvement in "Methods of Galvanizing," an error appears in the printed specification requiring correction as follows: Page 3, line 78, for the word "oxidization" read *oxidation*; and that the said Letters Patent should be read with this correction therein that the same may conform to the record of the case in the Patent Office.

Signed and sealed this 27th day of July, A. D., 1915.

[SEAL.]

R. F. WHITEHEAD,  
*Acting Commissioner of Patents.*